



US007122224B2

(12) **United States Patent**  
**Das et al.**

(10) **Patent No.:** **US 7,122,224 B2**  
(45) **Date of Patent:** **Oct. 17, 2006**

(54) **METHODS AND APPARATUS FOR TURBINE ENGINE COMPONENT COATING**

(75) Inventors: **Nripendra Nath Das**, West Chester, OH (US); **W. Michael Gmerek, Jr.**, West Chester, OH (US); **David W. Koch**, Pleasant Plain, OH (US)

(73) Assignee: **General Electric Company**, Schenectady, NY (US)

(\*) Notice: Subject to any disclaimer, the term of this patent is extended or adjusted under 35 U.S.C. 154(b) by 453 days.

(21) Appl. No.: **10/458,991**

(22) Filed: **Jun. 11, 2003**

(65) **Prior Publication Data**

US 2006/0141158 A1 Jun. 29, 2006

(51) **Int. Cl.**  
**B05D 1/32** (2006.01)

(52) **U.S. Cl.** ..... 427/282; 427/256; 427/248.1; 427/255.34; 118/504; 118/505

(58) **Field of Classification Search** ..... 427/300, 427/282, 252, 253, 248.1, 154; 118/504, 118/505

See application file for complete search history.

(56) **References Cited**

U.S. PATENT DOCUMENTS

6,146,696 A 11/2000 Das et al.

|                |         |                            |
|----------------|---------|----------------------------|
| 6,168,874 B1   | 1/2001  | Gupta et al.               |
| 6,224,673 B1   | 5/2001  | Das et al.                 |
| 6,253,441 B1 * | 7/2001  | Wheat et al. .... 29/527.2 |
| 6,326,057 B1   | 12/2001 | Das et al.                 |
| 6,332,926 B1   | 12/2001 | Pfaendtner et al.          |
| 6,332,931 B1   | 12/2001 | Das et al.                 |
| 6,334,907 B1   | 1/2002  | Das et al.                 |
| 6,440,496 B1   | 8/2002  | Gupta et al.               |
| 6,458,473 B1   | 10/2002 | Conner et al.              |
| 6,482,470 B1   | 11/2002 | Reeves et al.              |
| 6,485,655 B1 * | 11/2002 | Das et al. .... 216/45     |
| 6,560,870 B1   | 5/2003  | Das et al.                 |
| 6,579,567 B1   | 6/2003  | Das et al.                 |

\* cited by examiner

*Primary Examiner*—Timothy Meeks

*Assistant Examiner*—Howard Abramowitz

(74) *Attorney, Agent, or Firm*—William Scott Andes; Armstrong Teasdale LLP

(57) **ABSTRACT**

A method for processing a substrate article is provided. The method includes masking a first portion of the substrate article with a maskant that includes a formed graphite piece that overlays and contacts the first portion of the substrate such that a second portion of the substrate is not overlaid nor contacted by the maskant; and processing the substrate article such that a coating of material is deposited on the second portion of the substrate, and wherein the maskant facilitates preventing the coating from being deposited on the first portion of the substrate article.

**14 Claims, 3 Drawing Sheets**





FIG. 1



FIG. 2



FIG. 3

## METHODS AND APPARATUS FOR TURBINE ENGINE COMPONENT COATING

### BACKGROUND OF THE INVENTION

The invention relates generally to components of the hot section of gas turbine engines, and more particularly, to a process for depositing a coating onto a selective area of a turbine component.

In gas turbine engines, for example, aircraft engines, air is drawn into the front of the engine, compressed by a shaft-mounted rotary compressor, and mixed with fuel. The mixture is burned, and the hot exhaust gases are passed through a turbine coupled to a shaft. The flow of gas turns the turbine, which drives the compressor. The hot exhaust gases flow from the back of the engine, providing thrust that propels the aircraft forward.

During operation of gas turbine engines, at least some components within the engine, maybe in contact with high temperature gases. Such components may include, for example, blades, vanes, and nozzles used to direct the flow of the hot gases.

To facilitate shielding the metallic parts from the combustion gases, environmental coatings may be applied to the components. Such environmental coatings may be produced by holding the part to be coated at a temperature in an atmosphere that is rich in a certain element or elements, often aluminum. The elements diffuse onto the surface of the part and form a diffusion coating in a process known as diffusion aluminide. In one form, the environmental coating is fabricated from a diffusion cobalt aluminide, nickel aluminide or platinum aluminide. The diffusion aluminide coating surface forms an aluminum oxide scale when exposed to oxygen-containing atmospheres at elevated temperatures, thus facilitating increased resistance to additional high temperature oxidation.

At least some other known component coating processes demand labor-intensive processes. For example, when the component is a low pressure turbine (LPT) nozzle, known coating processes require a labor intensive masking process wherein a commercially available aluminum gettering masking tape is applied to the desired area of the turbine component. More specifically, the tape is affixed in place using a sheet metal strip. However, continued exposure to the high temperatures utilized by the coating process, may cause the sheet metal strip to warp, such that the strip fails to provide adequate support for the masking tape. As a result the masking tape may undesirably dislodge from the component during the aluminide coating process, and an undesired area of the turbine nozzle may be aluminized.

### BRIEF DESCRIPTION OF THE INVENTION

In one aspect, a method for processing a substrate article is provided. The method includes masking a first portion of the substrate article with a maskant that includes a formed graphite piece that overlays and contacts the first portion of the substrate such that a second portion of the substrate is not overlaid nor contacted by the maskant; and processing the substrate article such that a coating of material is deposited on the second portion of the substrate, and wherein the maskant facilitates preventing the coating from being deposited on the first portion of the substrate article.

In another aspect, a method for coating a gas turbine engine turbine engine nozzle with an environmental coating is provided. The method includes masking a first portion of the turbine engine nozzle with a maskant including a formed

graphite piece that overlies and contacts the first portion of the nozzle, such that a second portion of the nozzle remains exposed, and depositing a coating on the second portion of the nozzle without removing the maskant such that the maskant facilitates preventing the coating from being deposited on the first portion of the nozzle.

In yet another aspect, a coating mask for use in coating a substrate is provided. The mask includes a first interlocking segment end, an opposite second interlocking segment end and a body extending therebetween, each interlocking segment end is configured to interlock with a respective interlocking end of an adjacent segment such that a plurality of interlocking segments overlay a substrate article first portion. The body includes a formed graphite mask segment configured to isolate a portion of the substrate article from a coating atmosphere, and a contour surface shaped to conform to a first portion of the substrate article.

### BRIEF DESCRIPTION OF THE DRAWINGS

FIG. 1 is a cross-sectional side view of an exemplary gas turbine engine;

FIG. 2 is a perspective view of an exemplary low pressure turbine nozzle that may be used with a gas turbine engine, such as the gas turbine engine shown in FIG. 1;

FIG. 3 is a perspective view of an exemplary inner mask segment that may be used with the nozzle shown in FIG. 2;

### DETAILED DESCRIPTION OF THE INVENTION

Nickel-base superalloy components of gas turbines are sometimes coated with aluminum and then heated to diffuse the aluminum into the surface of the article. The aluminum-rich surface is oxidized to produce an adherent aluminum oxide scale on the surface of the article. The aluminum oxide scale is an effective barrier against further oxidation and corrosion of the component in service.

The aluminum coating is typically applied by a vapor phase deposition process. In one embodiment, aluminum containing a cobalt-aluminum donor alloy and a halide activator, such as aluminum fluoride gas, is contacted to the component surface under conditions such that the compound decomposes to leave a layer of aluminum deposited on the surface. The aluminum diffuses into the surface during the deposition and any post-deposition heat treatment, producing the aluminum-enriched surface region.

It is sometimes the case in such deposition processes that a first portion of the surface of the article is to be left uncoated, and a second portion of the surface of the article is to be coated with aluminum. In order to prevent deposition of aluminum from the aluminum-containing gas, the first (uncoated) portion of the surface of the article is physically covered with a mask. The mask prevents contact of the aluminum-containing gas to the first portion. These maskants are intended to prevent the coating vapors from reaching the surface of the article, and to prevent depletion of the alloy components from the surface of the first portion of the surface.

FIG. 1 is a cross-sectional side view of an exemplary gas turbine engine 10. In one embodiment, engine 10 is an F110/129 engine available from General Electric Aircraft Engines, Cincinnati, Ohio. Engine 10 has a generally longitudinally extending axis or centerline 14 extending in a forward direction 16 and an aft direction 18. Engine 10 includes a core engine 30 which includes a high pressure compressor 34, a combustor 36, a high pressure turbine 38,

and a power turbine or a low pressure turbine 39 all arranged in a serial, axial flow relationship. In an alternative embodiment, core engine 30 includes a compressor, a detonation chamber, and a turbine arranged in a serial, axial flow relationship. Engine 10 also includes a bypass duct 44 that surrounds core engine 30, and enables fluid flow to be routed downstream from core engine 30 rather than through core engine 30. In an alternative embodiment, engine 10 includes a core fan assembly (not shown). An annular centerbody 50 extends downstream from core engine 30 toward a variable geometry exhaust nozzle 54.

During operation, airflow enters engine 10 and fuel is introduced to core engine 30. The air and fuel are mixed and ignited within core engine 30 to generate hot combustion gases. Specifically, pressurized air from high pressure compressor 34 is mixed with fuel in combustor 36 and ignited, thereby generating combustion gases. Such combustion gases drive high pressure turbine 38 which drives high pressure compressor 34. The combustion gases are discharged from high pressure turbine 38 into low pressure turbine 39. The core airflow is discharged from low pressure turbine 39 and directed aftward towards exhaust nozzle 54.

FIG. 2 is a perspective view of an exemplary low pressure turbine nozzle 200 that may be used with a gas turbine engine, such as gas turbine engine 10 (shown in FIG. 1). Nozzle 200 includes a plurality of circumferentially-spaced airfoil vanes 202 coupled together by an arcuate radially outer band or platform 204, and an arcuate radially inner band or platform 206. More specifically, in the exemplary embodiment, each band 204 and 206 is integrally-formed with airfoil vanes 202.

In the exemplary embodiment, each airfoil vane 202 includes a first sidewall 208 and a second sidewall 210. First sidewall 208 is convex and defines a suction side of each airfoil vane 202, and second sidewall 210 is concave and defines a pressure side of each airfoil vane 202. Second sidewall 210 is joined to first sidewall 208 at a leading edge 212 and at an axially-spaced trailing edge (not shown) of each airfoil vane 202. More specifically, each airfoil trailing edge is spaced chordwise and downstream from each respective airfoil leading edge 212.

Second sidewall 210 and first sidewall 208 extend longitudinally, or radially outwardly, in span from radially inner band 206 to radially outer band 204. Additionally, second sidewall 210 and first sidewall 208 define a cooling cavity (not shown) within each airfoil vane 202. More specifically, the cooling cavity is bounded by an inner surface (not shown) of each airfoil sidewall, and extends through each band 204 and 206.

In the exemplary embodiment, nozzle 200 is fabricated from a nickel-base superalloy. "Nickel-base" as used herein means that the alloy contains more nickel by weight than any other element, for example, but not limited to, nickel-base superalloy, Rene 80. In alternative embodiments, other materials such as iron-base, cobalt-base or titanium-base alloys may be used.

Nozzle 200 may be of any operable shape, such as, for example, a gas turbine blade, a gas turbine vane, a gas turbine nozzle, a piece of tubing, a tool shape, a pump impeller, a pump rotor, a fan blade, or an element of electronic hardware. Nozzle 200 may be prepared by any operable approach known in the art, such as casting or forging. Nozzle 200 may be furnished in substantially its final shape and dimensions as the aluminide coating is thin and adds little to the dimensions of the article. In some cases, the article may instead be furnished slightly undersized to account for the thickness of the applied coating. A first

portion of nozzle 200 may be masked with a second portion of nozzle 200 unmasked and exposed.

In the exemplary embodiment, nozzle 200 is illustrated partially masked for a aluminide coating process. An arcuate band of a plurality of outer maskant segments 214 overlay and are in contact with an outer periphery of outer band 204. Each outer maskant segment 214 includes a first circumferential end 216 and a second, opposite circumferential end 218. Each end 216 and 218 includes an interlocking tab 220 and an interlocking recess 222. In the exemplary embodiment, a radially inner surface (not shown) of segment 214 is machined to conform dimensionally to a radial outer surface (not shown) of outer band 204. In an alternative embodiment, the radially inner surface of segment 214 is molded to conform to the radially outer surface of outer band 204.

An arcuate band of inner maskant segments 224 overlay and contact an inner periphery 226 of inner band 206. Each inner maskant segment 224 includes a first circumferential end 228 and a second, opposite circumferential end 230. Each end 228 and 230 includes an interlocking tab 232 and an interlocking recess 234. In the exemplary embodiment, a radially outer surface 236 of segment 224 is machined to conform dimensionally to a radially inner surface 226 of inner band 206. In an alternative embodiment, the radially outer surface 236 of segment 224 is molded to conform to the radially inner surface 226 of inner band 206.

During the coating process, segments 214 and 224 are assembled to overlay and contact outer band 204 and inner band 206 respectively. Each surface of segments 214 and 224 that contacts inner and outer band 204 and 206 respectively is formed to conform to band surface to facilitate preventing the coating atmosphere from contacting the portions of the bands 204 and 206 that are in contact with mask segments 214 and 224. The machined surfaces of the segments that conform to the surfaces of bands 214 and 224 obviate the need to seal the edges of the contact surfaces to facilitate preventing coating atmosphere from reaching masked surfaces of band 204 and 206. Interlocking tabs 220 and recesses 222 of segments are engaged to facilitate providing lateral support to each adjacent segment and to provide a tortuous path past ends 216 and 218. After coating and/or diffusion, the coated nozzle 200 may be cooled, and segments 214 and 224 may be removed and later reused.

Each graphite piece may be formed by molding or extruding and may be machined from a monolithic block of graphite that is formed in any manner as is known in the art.

FIG. 3 is a perspective view of an exemplary inner mask segment 224 that may be used with nozzle 200 (shown in FIG. 2). Segment 224 includes first end 228 and second end 230. Each end 228 and 230 includes interlocking tab 232 and interlocking recess 234. Tab 232 and recess 234 are configured to engage and interlock with a tab and recess on each end of adjacent segments. Radially outer surface 236 of segment 224 is formed to conform to a respective mating face on inner band 206 (shown in FIG. 2).

Although segments 214 and 224 are illustrated in association with a process for masking a turbine nozzle, it should be understood that the methods and apparatus described above may be used to mask articles of shapes and orientations different than those described herein. It is anticipated that freestanding and/or formed graphite maskants provide benefits that would accrue to articles of various shapes and orientations.

The above-described methods and systems for applying diffusion aluminide coating on a selective area of a turbine engine component is cost-effective and highly reliable for facilitating coating a portion of a component where a coating

is desired and for facilitating preventing the coating atmosphere from contacting a portion of the component where a coating is not desired. Specifically, the freestanding, dimensionally stable mask segments are reusable and easily handled and positioned to protect the portion desired to be free of coating. As a result, the methods and apparatus described herein facilitate fabrication and maintenance of components in a cost-effective and reliable manner.

Exemplary embodiments of combinations of gas turbine engine components and coating masks are described above in detail. The combinations are not limited to the specific embodiments described herein, but rather, components of each combination may be utilized independently and separately from other components described herein. Each combination component can also be used in combination with other system components.

While the invention has been described in terms of various specific embodiments, those skilled in the art will recognize that the invention can be practiced with modification within the spirit and scope of the claims.

What is claimed is:

1. A method for processing a substrate article comprising: masking a first portion of the substrate article with a maskant that includes a formed graphite piece that overlays and contacts the first portion of the substrate, such that a second portion of the substrate is not overlaid nor contacted by the maskant, wherein the formed graphite piece includes a plurality of graphite segments that each include a first interlocking end and an opposite second interlocking end, and wherein masking a first portion comprises interlocking each segment interlocking end with a respective interlocking end of an adjacent segment such that the plurality of interlocking segments form an annular ring; and processing the substrate article such that a coating of material is deposited on the second portion of the substrate, and wherein the maskant facilitates preventing the coating from being deposited on the first portion of the substrate article.
2. A method in accordance with claim 1 wherein masking a first portion of the substrate article comprises masking a first portion of the substrate article that is fabricated from at least one of an iron-base alloy, a nickel-base alloy, a cobalt-base alloy, and a titanium-base alloy.
3. A method in accordance with claim 1 wherein masking a first portion comprises masking the first portion of the substrate article with a maskant that includes a graphite piece formed of at least one of molded graphite and extruded graphite.
4. A method in accordance with claim 1 wherein masking a first portion comprises providing a dimensionally stable graphite piece including a surface that is machined to conform the first portion of the substrate article.
5. A method in accordance with claim 1 wherein the substrate article is a gas turbine nozzle that includes an annular inner ring, an annular outer ring, and at least one airfoil extending between the inner and outer ring and wherein masking a first portion comprises:

providing a plurality of arcuate inner ring masking segments that each include a contact face that substantially conforms to a contour of a radially inner periphery of the inner ring, said contact face directly contacts the radially inner periphery of the inner ring;

providing a plurality of arcuate outer ring masking segments that each include a contact face that substantially

conforms to contour of a radially outer periphery of the outer ring, said contact face directly contacts the radially outer periphery of the outer ring.

6. A method in accordance with claim 1 wherein processing the substrate article comprises depositing an aluminum coating on the second portion of the substrate.

7. A method in accordance with claim 1 wherein processing the substrate article comprises depositing the coating of material using a vapor phase process.

8. A method for coating a gas turbine engine turbine engine nozzle with an environmental coating, said method comprising:

masking a first portion of the turbine engine nozzle with a maskant including a formed graphite piece that overlies and contacts the first portion of the nozzle, such that a second portion of the nozzle remains exposed, wherein the formed graphite piece comprises a plurality of graphite segments that each include a first interlocking end and an opposite second interlocking end, and wherein masking a first portion of the turbine nozzle comprises interlocking each graphite segment interlocking end with a respective interlocking end of an adjacent segment such that the plurality of interlocking segments form an annular ring; and

depositing a coating on the second portion of the nozzle without removing the maskant such that the maskant facilitates preventing the coating from being deposited on the first portion of the nozzle.

9. A method in accordance with claim 8 further comprises providing a turbine engine nozzle fabricated from at least one of an iron-base alloy, a nickel-base alloy, a cobalt-base alloy, and a titanium-base alloy.

10. A method in accordance with claim 8 wherein masking a first portion comprises masking the first portion of the substrate article with a maskant including a graphite piece formed of at least one of molded graphite and extruded graphite.

11. A method in accordance with claim 8 wherein masking a first portion comprises masking the first portion of the substrate article with a maskant including a dimensionally-stable graphite piece that includes a contoured surface that substantially conforms to the first portion of the nozzle.

12. A method in accordance with claim 8 wherein the turbine nozzle includes an annular inner ring, an annular outer ring, and at least one airfoil extending between the inner and outer ring, and wherein masking a first portion comprises:

providing a plurality of arcuate inner ring masking segments that each include a contact face that substantially conforms to a contour of a radially inner periphery of the inner ring, said contact face directly contacts the radially inner periphery of the inner ring;

providing a plurality of arcuate outer ring masking segments that each include a contact face that substantially conforms to contour of a radially outer periphery of the outer ring, said contact face directly contacts the radially outer periphery of the outer ring.

13. A method in accordance with claim 8 wherein depositing a coating comprises depositing an aluminum coating on the second portion of the turbine engine nozzle.

14. A method in accordance with claim 8 wherein depositing a coating comprises depositing the coating by vapor phase processing.